

Jan. 5, 1971

J. E. KNEPP

3,553,074

COIL OF SHEET MATERIAL WAX-TISSUE LAMINATE IN WHICH A  
LUBRICANT IN THE WAX MIGRATES THROUGH THE  
TISSUE TO BE SHEET MATERIAL

Filed March 13, 1968

2 Sheets-Sheet 1

FIG. 1.



FIG. 2.



FIG. 3.



INVENTOR.  
JAMES E. KNEPP  
By *Abraham W. Hataler*  
Attorney

Jan. 5, 1971

J. E. KNEPP

3,553,074

COIL OF SHEET MATERIAL WAX-TISSUE LAMINATE IN WHICH A  
LUBRICANT IN THE WAX MIGRATES THROUGH THE  
TISSUE TO BE SHEET MATERIAL

Filed March 13, 1968

2 Sheets-Sheet 2

FIG. 4.



INVENTOR.  
JAMES E. KNEPP

By *Abraham H. Nather*

Attorney

## 1

3,553,074

### COIL OF SHEET MATERIAL WAX-TISSUE LAMINATE IN WHICH A LUBRICANT IN THE WAX MIGRATES THROUGH THE TISSUE TO BE SHEET MATERIAL

James E. Knepp, Pittsburgh, Pa., assignor to Aluminum Company of America, Pittsburgh, Pa., a corporation of Pennsylvania

Filed Mar. 13, 1968, Ser. No. 712,818

Int. Cl. B32b 15/12, 31/06

U.S. Cl. 161—223

6 Claims

### ABSTRACT OF THE DISCLOSURE

Texturing the surface of the sheet material-wax-tissue laminate by adding a lubricant to the wax which is coated on the sheet material prior to laminating with the tissue. The lubricant, which is preferably liquid at room temperature, migrates through the tissue layer to the surface of the layer of sheet material which becomes adjacent thereto when the laminate is coiled.

### BACKGROUND OF THE INVENTION

This invention relates to a sheet material-wax-tissue laminate. More particularly, it relates to improvement of the lubricant properties of the foil surface of a foil-wax-tissue laminate by supplying a texturant to the foil surface while the laminate is in coil form.

Sheet material, for example, foil laminate or laminated foil, is used for wrapping gum, candy, lozenges, cereal, cookies or the like. Heretofore, texturants or lubricants required to permit folding, forming or creasing of laminates without tearing or scuffing have been applied directly to the sheet material surface, for example, by application from a solvent which is evaporated. Such direct application has proved rather costly and has failed in many instances to provide as effective a lubricated surface as desired, as evidenced by such difficulties oftentimes encountered as breakage of foil during the wrapping operation, as in end tucking, traveling on guide rails or blocking of the foil upon unrolling from coils prior to packaging use. Therefore provision of a foil-wax-tissue laminate having an improved textured surface represents a highly desirable result.

### SUMMARY OF THE INVENTION

It is an object of this invention to provide a sheet material-wax-tissue laminate which has a sheet material surface of improved lubricant properties when the laminate is wound in coil form. It is a further object of this invention to provide a method of improving the lubricant properties of the sheet material-wax-tissue laminate. A still further object of this invention is to provide a sheet material surface which is resistant to blocking, that is, has a satisfactory degree of slip, when the material is unwound from coil form, and is resistant to scuffing and tearing when the foil is used in wrapping mints, candy, cereal or the like. These and other objects will be apparent from the description and claims which follow.

In accordance with this invention, in the manufacture of a sheet material laminate a texturant or lubricant is added to the laminating wax before the wax is applied to the sheet material. The major requirements of the texturant or lubricant according to my invention are (1) that it be compatible with the wax at temperatures above the wax melting point, (2) that it be semi-liquid or liquid, that is, fluid or mobile at room temperature, that is, at about 20-25° C. under ambient conditions, and (3) that it be capable of migrating through the tissue layer to texture the surface of the sheet material which becomes adjacent

## 2

to the tissue layer when the laminate is wound in coil form. Useful texturants or lubricants according to my invention include fatty acids and their esters, mineral and vegetable oils, and the like. Such may be used singly or in admixture. One advantage of this use of texturant in the wax is that the wax containing the texturant may be applied to the foil without need for new equipment or costly solvents, for example, by a roller used to apply the wax from a melt contained in a pan or the like before it is laminated with tissue.

When the laminate is wound in coil form and then stored, the texturant, due to its mobility or migrating characteristic at room temperature, is taken up or absorbed by the tissue, which acts much like a wick, and is transferred to the surface of foil adjacent the tissue layer, thereby lubricating it. Concentration of lubricant in wax is controlled such that a sufficient amount migrates through the tissue to provide lubricant properties and machinability to the adjacent coiled foil surface. Concentrations in the range of 0.5 to about 6% by weight, based upon the weight of the wax have proven beneficial with the optimum concentration being about 1.5 to about 2.5%. The lubricant may be dissolved in the wax by heating, preferably to a temperature of about 160-200° F., the optimum temperature being about 175-185° F. The wax containing the lubricant is preferably applied to the foil within about this same temperature range.

The base sheet material of this invention is preferably metal. A metal foil, preferably aluminum, is preferred. By 30 foil we mean any thin sheet metal or metal alloy having a thickness of a few thousandths of an inch or less, usually about 0.006 inch or less, preferably from about 0.0003 to 0.0004 inch. Some of the aluminum foils useful according to this invention are those containing at least about 99% 35 by weight aluminum and up to about 1% by weight silicon and iron or other alloying elements. Copper, manganese, zinc and the like may be also present in such aluminum alloys in amounts up to about 0.1 each. Annealed or dead soft temper aluminum alloys may be laminated according to the invention.

To be useful in containing and transferring texturants according to my invention, the laminating waxes may be of the microcrystalline or paraffin variety, and preferably of strong laminating and heat seal strengths. Microcrystalline wax is preferred, but the preferred microcrystalline wax may contain 50% or more paraffin. The laminating wax may contain other minor ingredients such as rubber, for example, butyl rubber, a copolymer, for example, ethylene vinyl acetate and ethylene isobutyl acrylates, and resins, for example, terpene or wood resin, or like additives. Preferred amount of wax in coating the foil according to the invention is from about 3 to about 25 lbs. per ream.

For the tissue to have the desired properties for use in the laminate of this invention it should weigh from 55 about 8 to about 20 pounds per 3,000 square feet, be porous and of a sufficiently low density to permit wicking and migration of the texturant or lubricant from the wax and through the tissue to the adjacent foil surface.

In providing the desired lubricant properties to the 60 foil surface according to my invention, the texturant, when transferred from the wax via the tissue to the foil surface when the foil is in coil form, in furnishing the desired anti-blocking or slip properties causes a substantial reduction in coefficient of friction, viz., from as high 65 as about 1.0 down to a minimum of about 0.15 and down to a range of from about 0.40 to about 0.20, preferably from about 0.35 to about 0.25. The amount of lubricant which reaches the foil surface via the tissue layer upon storage of the foil in coil form is from about 0.0005 70 mg./in.<sup>2</sup> to about 0.1 mg./in.<sup>2</sup>, preferably from about 0.0025 mg./in.<sup>2</sup> to about 0.05 mg./in.<sup>2</sup>.

## 3

Texturants useful according to the invention in providing the desired lubricant properties, strength and adhesion when transferred to the foil surface from the laminating wax include lubricants such as butyl stearate, methyl stearate, methyl oleate, methyl myristate, mineral oil, glyceryl trioleate, glyceryl mono-oleate, acetylated monoglycerides, castor oil, dioctyl sebacate, polyethylene sorbitan mono-oleate, silicones, soybean oil, corn oil, cottonseed oil, coconut oil, sesame seed oil and the like. Highly effective among these are butyl stearate, cottonseed oil, soybean oil, coconut oil, sesame seed oil and mineral oil.

The time required for transfer of the lubricant from the laminating wax in which it is applied to the foil surface through the tissue to the foil surface adjacent the tissue layer is from about 1 hour to about 24 hours.

## BRIEF DESCRIPTION OF THE DRAWINGS

For a more detailed description of the invention reference is made to the accompanying drawings, which illustrate a preferred embodiment of the invention.

## DESCRIPTION OF THE PREFERRED EMBODIMENT

## In the drawings:

FIG. 1 is a horizontal cross-section of the laminated foil of the invention showing the lubricant 2 contained in the wax layer 4 on the foil layer 6 prior to storage and migration through the tissue layer 8.

FIG. 2 is a cross-section of the laminated foil of the invention in coil form showing the lubricant 2 contained in the wax layer 4 on the foil layer 6 prior to migration through the tissue layer 8.

FIG. 3 is a cross-section of the laminated foil of the

## 4

invention in coil form showing the lubricant 2 in the form of a layer or coating on the surface of the foil layer 6 after migration from the wax layer 4 through the tissue layer 8.

FIG. 4 is a schematic representation of one process embodiment by which my foil laminate containing lubricant in the wax may be prepared according to the present invention. In FIG. 4, foil 10 is unwound from coil 12 and conducted via roll 14 over turning roll 16, which applies wax containing lubricant 18 from wax pan 20. After passing over metering bar 22 the wax coated foil 24 is laminated with tissue 26 from coil 28 by passing through the nip formed between rolls 30 and 32 and then wound as laminated foil 34 on coil 36 after passing over chill roll 38.

The following examples are illustrative of the invention.

## EXAMPLE I

Representative texturants useful according to this invention were dissolved in wax and the wax applied to aluminum foil of 0.0003 to 0.00035 inch gauge. The foil was then laminated with tissue and stored in coiled form. The textured foil surfaces were then evaluated at various time intervals for coefficient of friction (COF), both static and kinetic, textured surface to textured surface, on a conventional moving web-stationary sled apparatus such as described in Bakelite Flexible Packaging Materials Technical Release No. 2, August 1955. The durability or thumb rub resistance of the textured foil was determined by rubbing the two surfaces against each other under moderate thumb pressure with a rub amplitude of approximately two inches. Results are reported in Table 1.

TABLE 1

| Texture material                                       | Percent by wt. | Coefficient of friction (static/kinetic), foil-foil, moving web |           |           | Thumb rub, foil-foil, average of 2 individuals |        |        | 10 days |
|--------------------------------------------------------|----------------|-----------------------------------------------------------------|-----------|-----------|------------------------------------------------|--------|--------|---------|
|                                                        |                | 1 day                                                           | 3 days    | 7 days    | 1 day                                          | 3 days | 7 days |         |
| None, plain foil surface                               |                | 1.0/1.0-9                                                       | 1.0/1.0-9 | 1.0/1.0-9 | 0                                              | 0      | 0      |         |
| Butyl stearate                                         | 1/2            | .90/.66                                                         | .82/.65   | .75/.40   | 0                                              | 0      | 0      |         |
|                                                        | 1              | .70/.49                                                         | .30/.60   | .32/.42   | 0                                              | 1      | 1      |         |
|                                                        | 2              | .31/.42                                                         | .22/.27   | .20/.25   | 3-5                                            | 5-7    | 11     |         |
|                                                        | 4              | .25/.27                                                         |           | .19/.24   |                                                |        |        |         |
|                                                        | 6              | .23/.22                                                         |           | .19/.21   |                                                |        |        |         |
|                                                        | 1              | .55/.35                                                         |           | .35/.24   |                                                |        |        | 4-5     |
|                                                        | 1              | .31/.42                                                         | .27/.28   | .25/.25   |                                                |        |        | 3-5     |
|                                                        | 1 1/2          | .30/.31                                                         |           | .29/.28   |                                                |        |        | 3       |
|                                                        | 1 1/2          | .27/.27                                                         | .27/.27   | .24/.24   |                                                |        |        | 3-5     |
|                                                        | 2              | .31/.24                                                         |           | .29/.27   |                                                |        |        | 3-4     |
|                                                        | 2              | .29/.33                                                         | .26/.27   | .24/.26   |                                                |        |        | 3-5     |
| Wesson oil (cottonseed)                                | 2              | .75/.52                                                         | .38/.35   | .29/.31   | 0.1                                            | 1-3    | 2-5    |         |
| Acetylated monoglyceride                               | 2              | .29/.29                                                         | .25/.24   | .24/.24   | 4-7                                            | 4-9    | 4-10   |         |
|                                                        | 2              | .31/.26                                                         | .26/.25   | .23/.24   | 5-13                                           | 5-11   | 5-10   |         |
|                                                        | 1              | .31/.27                                                         | .30/.29   | .25/.26   | 3-5                                            | 2-4    | 2-7    |         |
|                                                        | 1 1/2          | .34/.26                                                         | .25/.26   | .23/.24   | 1-5                                            | 3-8    | 3-9    |         |
| 75% acetylated monoglyceride, 25% dioctyl sebacate     | 2              | .32/.31                                                         | .29/.28   |           | { 3-8                                          | 4-8    | 3-9    |         |
|                                                        |                |                                                                 |           |           | { 0-3                                          | 2-5    |        |         |
| Acetylated monoglyceride                               | 1              | .29/.26                                                         | .27/.27   | .28/.25   | { 3-5                                          | 2-6    | 2-4    |         |
|                                                        | 1 1/2          | .30/.27                                                         | .27/.26   | .27/.25   | 4-5                                            | 4-6    | 3-8    |         |
|                                                        | 2              | .30/.25                                                         | .24/.25   | .26/.25   | 5-8                                            | 5-12   | 4-10   |         |
|                                                        | 2              | .50/.36                                                         | .35/.34   | .35/.38   |                                                |        |        | 10-21   |
| 25% butyl stearate plus 75% mineral oil                | 2              | .30/.26                                                         | .28/.26   | .27/.27   | { 4-9                                          | 3-6    | 2-8    | 0-2     |
| 25% dioctyl sebacate plus 75% acetylated monoglyceride | 2              |                                                                 |           |           | { 0                                            | 1/2-6  | 2-7    |         |
| Wesson oil (cottonseed)                                | 4              | .68/.55                                                         | .34/.35   | .29/.27   | 0                                              | 1/2-4  | 2-6    |         |
|                                                        | 3              | .46/.52                                                         | .30/.29   | .27/.27   | 1/2-3                                          | 1-4    | 3-5    |         |
|                                                        | 2              | .30/.33                                                         | .29/.32   | .31/.26   | 1/2-4                                          | 0.3    | 2-4    |         |
|                                                        | 1              | .31/.36                                                         | .35/.35   | .31/.28   | 0-1                                            | 0-3    | 2-5    |         |
| Wesson oil plus butyl stearate (3:1)                   | 2              | .34/.47                                                         | .31/.36   | .30/.28   | 3-6                                            | 5-7    | 2-6    |         |
| Methyl oleate                                          | 2              | .23/.23                                                         | .25/.26   | .24/.23   | 2-6                                            | 2-4    |        |         |
| Glyceryl trioleate                                     | 2              | .28/.30                                                         | .26/.24   |           |                                                |        |        |         |
| Glyceryl monooleate plus Wesson oil (1:3)              | 2              | .40/.43                                                         | .33/.31   |           | { 0-1/2                                        | 1-3    |        |         |
| Glyceryl monooleate plus Wesson oil (1:3)              | 1              | .43/.51                                                         | .28/.31   |           | { 1                                            | 2-3    |        |         |

## EXAMPLE II

Textured aluminum foil laminates were prepared substantially as in Example I using .00035 inch foil, 16-lb. wax, 8.5-lb. tissue, and several different lubricants (dissolved in the wax). Evaluations were performed for coefficient of friction and thumb rubs (foil to foil) after aging for various periods, a sufficient amount of lubricant having migrated through the tissue to the adjacent foil surface upon winding of the foil in coils to reduce the coefficient of friction to the values indicated in Table 2.

TABLE 2

| Texture material                     | Percent by wt. | Days after fabricating | Coefficient of friction static/kinetic foil-foil | Thumb rubs (foil-foil) |
|--------------------------------------|----------------|------------------------|--------------------------------------------------|------------------------|
| None, plain foil surface             | 0              | 44                     | 1.0/1.0-9                                        | 0                      |
| Butyl stearate                       | 1½             | 44                     | .23/.24                                          | 4-6                    |
|                                      | 1½             | 44                     | .25/.26                                          | 3-4                    |
|                                      | 2              | 44                     | .22/.23                                          | 3-4                    |
|                                      | 2              | 44                     | .22/.23                                          | 3-4                    |
| Wesson oil (cottonseed oil)          | 2              | 21                     | .27/.25                                          | 3-4                    |
| Wesson oil                           | 2              | 14                     | .31/.27                                          | 3-4                    |
| Wesson oil plus butyl stearate (3:1) | 1              | 14                     | .31/.27                                          | 3-5                    |
| Glyceryl trioleate                   | 2              | 14                     | .28/.26                                          | 4                      |
|                                      | 2              | 10                     | .26/.26                                          | 2-3                    |

## EXAMPLE III

Textured aluminum foil (.00035 inch gauge) laminates were prepared substantially as in Example I using butyl stearate and cottonseed oil as lubricants. Physical properties and functional properties confirming transfer of lubricant from the wax through the tissue to the foil surface are recorded in Table 3.

TABLE 3.—FUNCTIONAL PROPERTIES

| Texture     | Structure            |                                      |        | Coefficient of friction moving web |         |                |         | Thumb rubs, No. strokes |  |
|-------------|----------------------|--------------------------------------|--------|------------------------------------|---------|----------------|---------|-------------------------|--|
|             | Wax (per ream), lbs. | Texture weight, mg./in. <sup>2</sup> | Tissue | Foil-foil                          |         | Foil-stainless |         |                         |  |
|             |                      |                                      |        | Static                             | Kinetic | Static         | Kinetic |                         |  |
| Sample No.: |                      |                                      |        |                                    |         |                |         |                         |  |
| 1           | Butylstearate        | 14.6                                 | 8.5    | .001                               | .29     | .27            | .26     | .26 3-5                 |  |
| 2           | Cotton seed oil      | 14.8                                 | 8.5    | .001                               | .24     | .23            | .23     | .26 4-7                 |  |

## EXAMPLE IV

Various representative lubricants useful according to the invention were added to laminating wax at 2% concentrations and aluminum foil coated therewith, laminated with tissue and rolled in coils substantially as in Example I, using 14 lb. wax per ream. After varying periods of storage in coil form at ambient temperatures, the foil surfaces were examined and analyzed to test migration and transfer of lubricants and amount of resulting texturing of the foil surfaces. Coefficient of friction and thumb rub tests were performed. Table 4 contains the results of the evaluations.

TABLE 4

| 14 lb./ream wax containing 2% by weight additive | Coefficient of friction, foil to foil, moving web (static/kinetic) |         |         |         | Thumb rub, foil to foil, average of three individuals |        |        |         |
|--------------------------------------------------|--------------------------------------------------------------------|---------|---------|---------|-------------------------------------------------------|--------|--------|---------|
|                                                  | 2 days                                                             | 5 days  | 7 days  | 28 days | 2 days                                                | 5 days | 7 days | 28 days |
| Edible soybean oil                               | .38/.38                                                            | .34/.34 | .33/.34 | .26/.26 | 1½-2                                                  | 2-2½   | 2½-3   | 1½-2½   |
| Refined corn oil                                 | .46/.47                                                            | .33/.35 | .29/.29 | .26/.26 | 1½-2                                                  | 2½-3   | 2½-3   | 2½-3    |
| Cottonseed cooking oil                           | .43/.44                                                            | .35/.35 | .30/.30 | .26/.26 | 2-3                                                   | 3-3½   | 3-4    | 3-3½    |
| Coconut oil                                      | .41/.43                                                            | .36/.36 | .31/.31 | .26/.26 | 1-2                                                   | 1½-2½  | 1½-2½  | 1½-2½   |
| Sesame seed oil                                  | .47/.49                                                            | .35/.35 | .29/.29 | .25/.24 | 1-2½                                                  | 2-3    | 2½-3½  | 3-3½    |

While the invention has been described in terms of preferred embodiments, the claims appended hereto are intended to encompass all embodiments which fall within the spirit of the invention.

Having thus described my invention and certain embodiments thereof, I claim:

1. A coil of laminated relatively impermeable base sheet material wound in repeating order outwardly comprising from the axial core of said coil respective layers of said sheet material, wax, tissue and lubricant, said lubricant being compatible with the wax at temperatures

above the melting point thereof and mobile at room temperature and said lubricant layer being characterized by having resulted from said lubricant having been present in a sufficient amount to migrate from said wax through said tissue and thereby act as a lubricant for the next outwardly adjacent surface of the repeating sheet material layer.

2. The coil of claim 1 wherein the sheet material is aluminum foil, the wax is microcrystalline wax, paraffin wax or a blend of the two, the lubricant is selected from the group consisting of fatty acids, esters of fatty acids and mineral and vegetable oils, and the lubricant comprises from about 0.0005 mg. to about 0.1 mg. per square inch of the next outwardly adjacent surface of the repeating sheet material layer.

3. The coil of claim 1 wherein the sheet material is aluminum foil, the wax is microcrystalline wax, paraffin wax or a blend of the two, the lubricant is selected from the group consisting of fatty acids, esters of fatty acids and mineral and vegetable oils, and the coefficient of friction of the next outwardly adjacent surface of the repeating sheet material layer is from about 0.20 to about 0.40.

4. A method of texturing the surface of a laminated sheet material which comprises coating a sheet material base with wax containing a lubricant which is compatible with the wax at temperatures above the melting point thereof and mobile at room temperature, laminating said sheet material base coated with said wax containing a lubricant with a porous tissue, and winding the resulting laminated sheet material in a coil, said lubricant being present in an amount sufficient upon storage of said coil

to enable said lubricant to migrate through said tissue and texture the surface of the sheet material adjacent said tissue with a resultant lowering of the coefficient of friction of said surface.

5. The method of claim 4 wherein the lubricant contained in the wax is from about 0.5 to about 6% by weight of said wax of a substance selected from the group consisting of fatty acids, esters of fatty acids, and mineral and vegetable oils, the wax is microcrystalline wax, paraffin wax or a blend of the two, the sheet material is aluminum foil, the tissue has a weight of from about 8 to about 20 pounds per 3,000 square feet, and the lubricant is present in the wax in an amount sufficient to

reduce the coefficient of friction of the surface of the aluminum foil adjacent the tissue to between about 0.20 and 0.40 and is selected from the group consisting of fatty acids, esters of fatty acids, and mineral and vegetable oils.

6. A method of lowering the coefficient of friction of the surface of aluminum foil which comprises dissolving from about 0.5 to about 6% by weight of a lubricant in a microcrystalline or paraffin wax having a weight of from about 3 to about 25 lb./ream at a temperature of from about 160° to about 200° F., said lubricant being com-

patible with said wax at temperatures above the melting point of the wax and mobile at room temperature, coating aluminum foil at said temperature of from about 160° to about 200° F. with the resulting wax containing said lubricant, laminating said foil with a porous tissue having a weight of from about 8 to about 20 lb./ft.<sup>2</sup>, said lubricant being present in an amount sufficient upon storage of the resulting laminate in coil form to migrate differentially from said wax through said porous tissue, and within from about 1 to about 24 hours transferring an amount of said lubricant from said wax through said tissue sufficient to reduce the coefficient of friction of foil surface adjacent said laminating tissue by thumb rub test, foil to foil, from substantially no rubs to about 2.0 to 4.0.

## References Cited

## UNITED STATES PATENTS

|   |           |         |                 |       |         |
|---|-----------|---------|-----------------|-------|---------|
| 5 | 2,726,979 | 12/1955 | Grant           | ----- | 161—223 |
|   | 2,783,161 | 2/1957  | Padgett         | ----- | 106—207 |
|   | 2,847,367 | 8/1958  | Walsh           | ----- | 106—270 |
|   | 3,373,915 | 3/1968  | Anderson et al. | ----- | 161—223 |

JOHN T. GOOLKASIAN, Primary Examiner

10 M. E. McCAMISH, Assistant Examiner

## U.S. Cl. X.R.

156—184; 161—235, 220